

# United States Patent Office

3,484,345  
Patented Dec. 16, 1969

1

3,484,345

## NICKEL ELECTROPLATING

Raymond F. Nambride, Paris, France, assignor to Enthone, Incorporated, West Haven, Conn., a corporation of Connecticut  
No Drawing. Filed Feb. 7, 1967, Ser. No. 614,402  
Int. Cl. C23b 5/46, 5/08  
U.S. Cl. 204—49

27 Claims

### ABSTRACT OF THE DISCLOSURE

This invention is concerned with baths or solutions for electroplating of nickel and containing, as brightness and leveling additive, one or more reaction products of an aldehyde with a nuclear substituted heterocyclic nitrogen-containing compound. Additionally this invention is concerned with brightening and leveling additive compositions for nickel electroplating baths, and with a method for electroplating bright, level nickel deposits.

This invention relates to electrolytic nickel plating and more particularly to new and improved baths and method for the electroplating of bright, level nickel deposits. Additionally this invention is concerned with brightness and leveling additive compositions for nickel electroplating baths.

In accordance with the present invention, it has been found that bright, level nickel electrodeposits are obtained on the object, article or surface being plated by adding or incorporating into the acidic aqueous nickel electroplating solution an effective amount of one or more reaction products of an aldehyde hereinafter specified with a nuclear substituted heterocyclic nitrogen-containing compound of the formula



wherein R<sub>1</sub> and R<sub>2</sub> separately are each hydrogen and taken together are



and m is an integer from 0 to 1, m being zero when R<sub>1</sub> and R<sub>2</sub> taken together are as aforesaid, all substituents of such substituted heterocyclic compound being on carbon atoms of the heterocyclic nucleus with the nitrogen atom of the cyclic nucleus being unsubstituted. The aldehyde or aldehydes which react with the nuclear substituted heterocyclic compound to form the reaction product or products aforesaid are selected from those of the formula



wherein R is from the group consisting of lower alkyl, 65 alkenyl, lower alkynyl, hydroxymethyl, trichloromethyl, furfuryl, i.e.



2

and carboethyl, i.e.



5 The nickel plating bath solution herein also contains nickel sulfate and/or nickel chloride, preferably both such nickel salts, water, and preferably a buffering agent, with boric acid the preferred buffering agent. The reaction product or products herein of the aldehyde and substituted heterocyclic nitrogen-containing compound give good results as a brightener and especially good results as a leveling agent.

10 The aldehydes of the formula supra include, for example, propargylic aldehyde, chloral, furfural, acetaldehyde, butyraldehyde, propionaldehyde, valeraldehyde, acrolein, citronellal, crotonaldehyde, tigraldehyde, glycolaldehyde, and succinaldehyde. Citronellal is a mixture of the stereoisomeric aldehydes:



and



15 The exemplary lower alkyl aldehydes set forth supra are characterized by being 1-4C alkyl aldehydes, and the exemplary alkenyl aldehydes by having mono- or di-olefinically unsaturated alkenyl groups with from 2-9 carbon atoms in the alkenyl group. Any lower alkynyl aldehyde is utilizable herein for reaction with the substituted heterocyclic nitrogen-containing compound to obtain the additive compounds herein, and by "lower alkynyl" as used herein is meant mono-acetylenically unsaturated alkynyl having from 2-8 carbon atoms in the alkynyl group. The lower alkynyl aldehydes are the preferred aldehydes herein with propargylic aldehyde being preferred among such aldehydes, for reaction with the preferred nuclear-substituted nitrogen-containing heterocyclic compounds hereinafter disclosed, for obtaining the preferred reaction product additive compounds herein.

20 Exemplary of the nuclear substituted heterocyclic nitrogen-containing compounds are  $\alpha$ -picoline or  $\alpha$ -methylpyridine



25  $\gamma$ -picoline or  $\gamma$ -methylpyridine



30 35 quinaldine or 2-methylquinoline



40 45 50 55 60 65 70 75 80 85 90 95 and  $\alpha, \gamma$ -lutidine,  $\alpha, \alpha'$ -lutidine and lipidine or 4-methylquinoline. The  $\alpha$ -methylpyridine,  $\gamma$ -methylpyridine and 2-methylquinoline are the preferred nuclear substituted nitrogen-containing heterocyclics for reaction with the preferred aldehydes previously disclosed herein to obtain the preferred reaction product additives herein.

The methyl group or groups of the nuclear substituted heterocyclic nitrogen-containing compounds herein are preferably linked to the alpha ring carbon and/or gamma ring carbon, relative to the ring nitrogen atom, which correspond to the 2 and 4 positions. Methyl groups linked to the ring carbons in such positions are very reactive.

The reaction product of the aldehyde and the substituted heterocyclic nitrogen-containing compound containing the pyridine ring herein is added or incorporated into the nickel electroplating bath herein in an effective amount, sufficient to obtain bright, level nickel electro-deposits. The effective amount added to the nickel electroplating bath or solution to obtain such results is usually a minor amount, preferably from about 5-200 milligrams of such reaction product or products per liter of the nickel electroplating bath or solution. Instead of the addition to the plating solution of the reaction product or products of a single aldehyde with a single heterocyclic nitrogen-containing compound, the reaction product or products of two or more aldehydes herein with one or more of the heterocyclic nitrogen-containing compounds herein can be added to the plating solution as the brightening and leveling additive.

The aldehyde herein reacts with the nuclear substituted heterocyclic nitrogen-containing compound in accordance with the following:



wherein  $\text{R}$ ,  $\text{R}_1$ ,  $\text{R}_2$  and  $m$  are as aforesaid. The substituent containing the hydroxyl radical of the Type I compound or the substituent containing the olefinic double bond of the Type II compound are preferably linked to the alpha or gamma carbon with respect to the nitrogen of the cyclic nucleus, and the methyl group substituent when present is linked to that alpha or gamma carbon of the cyclic nucleus not bonded to the hydroxy- or olefinic double bond-containing substituent. The last-mentioned methyl group substituent when present can be the  $-\text{CH}_3$  group as such or the  $-\text{CH}_2\text{CHOH---R}$  or  $\text{CH}=\text{CH---R}$  group (wherein  $\text{R}$  has the meaning aforesaid) resulting from the reaction of the di-methyl substituted heterocyclic nitrogen-containing compound with the aldehyde. And by such  $-\text{CH}_3$  group substituent when present in the Type I or Type II reaction product compound herein is meant either the  $-\text{CH}_3$  group per se, the  $-\text{CH}_2\text{---CHOH---R}$  group, or the  $-\text{CH}=\text{CH---R}$  group, wherein  $\text{R}$  has the meaning aforesaid. The condensation reaction of the substituted heterocyclic nitrogen-containing compound and the aldehyde to produce the hydroxylated compound of Type I, is effected at temperature usually in the range of about  $20^\circ\text{C}$ .- $40^\circ\text{C}$ . The intra-molecular dehydration of the Type I compound to form the compound of Type II having the olefinically unsaturated nuclear substituent occurs at higher temperature usually in the range of about  $60^\circ\text{C}$ .- $100^\circ\text{C}$ . The reaction product that is added to or incorporated into the nickel plating bath herein is either the Type I compound supra or the Type II compound supra, or a mixture of the Type I and Type II compounds when the temperature of the reaction mixture has first been within the lower temperature range aforesaid for the Type I compound, and subsequently reaches for an

5 insufficient time to convert all Type I compound to Type II compound the higher range of temperature aforesaid for the Type II compound. The following equations set forth the reaction of  $\alpha$ -picoline and the aldehyde to form the Type I compound and the intramolecular dehydration of the Type I compound to form the Type II compound:



20 wherein  $\text{R}$  is as aforesaid.

The Type I compound and/or Type II compound supra is added to a nickel electroplating bath such as, for example, that containing:

|                            | G./I.   |
|----------------------------|---------|
| 25 $\text{NiSO}_4$         | 250-400 |
| 25 $\text{NiCl}_2$         | 10-200  |
| 25 $\text{H}_3\text{BO}_3$ | 10-40   |

and the nickel electrodeposit obtained by electrolyzing the bath between the anode and cathode, with the metallic surface or article to be plated the cathode, at a bath temperature usually in the range of about  $20^\circ\text{C}$ .- $70^\circ\text{C}$ ., preferably about  $60^\circ\text{C}$ ., a current density in the range of usually about 10-100 amperes per square foot, preferably about 50 a.s.f., a bath pH (electrometric preferably between 3.0 and 5.5, and with preferably cathode agitation or compressed air agitation of the electrolyte in the vicinity of the cathode.

Exemplary of the Type I and Type II compounds herein are set forth hereafter. These compounds are added to the nickel plating bath singly, i.e. either the Type I or Type II compound separately, or as a mixture of the Type I and Type II compounds.



60 Product of reaction between  $\gamma$ -methylpyridine and chloral



5

Product of reaction between 2-methylquinoline and chloral

Type II



Type I

Product of reaction between  $\alpha$ -methylpyridine and propargylic aldehyde

Type II



Type I

Product of reaction between  $\gamma$ -methylpyridine and propargylic aldehyde

Type II



Type I



Product of reaction between 2-methylquinoline and propargylic aldehyde

Type II



Type I

Product of reaction between  $\alpha$ -methylpyridine and furfural

Type II



Type I

Product of reaction between  $\gamma$ -methylpyridine and furfural

Type II



Type I

6



5

Product of reaction between 2-methylquinoline and furfural

Type II



Type I

Product of reaction between  $\alpha$ -methylpyridine and acetaldehyde

Type II



Type I

Product of reaction between  $\alpha$ -methylpyridine and acetaldehyde

Type II



Type I

Product of reaction between  $\alpha$ -methylpyridine and butyraldehyde

Type II



Type I

Product of reaction between  $\alpha$ -methylpyridine and butyraldehyde

Type II



Type I



75

Product of reaction between  $\alpha$ -methylpyridine and acrolein

Type II



Type I



Product of reaction between  $\alpha$ -methylpyridine and acrolein

Type II



Type I



Type I



Product of reaction between  $\alpha$ -methylpyridine and citronellal

Type II



Type I



Product of reaction between  $\alpha$ -methylpyridine and citronellal

Type II



Type I



5 Product of reaction between  $\alpha$ -methylpyridine and tiglaldehyde

Type II



10 Type I



20 Product of reaction between  $\gamma$ -methylpyridine and tiglaldehyde

Type II



30 Type I



35 Product of reaction between  $\alpha$ -methylpyridine and crotonaldehyde

Type II



40 Type I



45 Product of reaction between  $\gamma$ -methylpyridine and crotonaldehyde

Type II



Type I



60 Type II



70 Type I



Product of reaction between  $\gamma$ -methylpyridine and glycolaldehyde

Type II



Type I



Product of reaction between  $\alpha$ -methylpyridine and succinaldehyde

Type II



Type I



Product of reaction between  $\gamma$ -methylpyridine and succinaldehyde

Type II



Type I



Product of reaction between 2-methylquinoline and acetaldehyde

Type II



Type I



Product of reaction between 2-methylquinoline and butyraldehyde

Type II



Type I



Product of reaction between 2-methylquinoline and acrolein

Type II



Type I



Product of reaction between 2-methylquinoline and citronellal

Type II



Type I



Product of reaction between 2-methylquinoline and tigaldehyde

Type II



Type I



Product of reaction between 2-methylquinoline and crotonaldehyde

Type II



Type I



Product of reaction between 2-methylquinoline and glycolaldehyde

Type II



Type I



Product of reaction between 2-methylquinoline and succinaldehyde

Type II



The foregoing enumeration of the Type I and Type II reaction products is exemplary and a partial listing only in the interest of avoiding prolixity.

The substituted heterocyclic compound reaction products or products of the aldehyde and nuclear-substituted

nitrogen-containing heterocyclic compound can be added to the nickel plating bath either as such, or when combined or mixed together with an inert diluent or carrier as an additive agent or composition. By "inert" is meant a diluent or carrier which is compatible and non-reactive or substantially non-reactive with the other constituents of the additive composition and electroplating bath to the material detriment of the additive and bath. The diluent or carrier may or may not itself have a function in the plating bath. Exemplary of the inert diluent or carrier is an inert liquid solvent such as, for instance, an aqueous liquid, e.g. water. However any inert liquid solvent which is compatible with the other ingredients of the electroplating bath can be utilized. An inert solid diluent or carrier can also be employed, for instance, sodium lauryl sulfate as powder, crystals or flakes, and which functions as an anti-pit, or saccharin in powder or crystal form and which functions as stabilizer for the bath. The amounts of the nuclear substituted heterocyclic compound reaction product or products and diluent or carrier in such additives can be varied over wide ranges, for instance a weight ratio of diluent to reaction product or total reaction products within the ratio range of about 40:1 to 3:1 respectively.

The reaction product of the aldehyde and substituted heterocyclic nitrogen-containing compound is preferably utilized in the nickel electroplating bath herein in combination with another or second brightening agent, which cooperates with such reaction product brightening agent in producing bright nickel deposits which are ductile as well as level. As the second or cooperating brightening agent is one or more of an organic sulfur- and oxygen-containing compound. Exemplary of such organic sulfur- and oxygen-containing compounds are aryl sulfonic acids and sulfonates, aryl sulfonamides and sulfonimides, mono-nuclear aryl sulfonic acids, unsaturated aliphatic sulfonic acids, heterocyclic sulfonic acids, and aryl sulfones. The aromatic or aryl sulfonic acids and sulfonates include both mononuclear and binuclear aryl sulfonic acids and sulfonates, with the aryl radical being of the benzene or naphthalene series. The sulfonates include the mono-, di- and tri-sulfonates of the benzene and naphthalene series of compounds. Exemplary of such organic sulfur compound brighteners are benzene mono- and disulfonic acids, 1,5-naphthalene disulfonic acid, 2,7-naphthalene disulfonic acid, 1,3,6-naphthalene trisulfonic acid, sodium benzenemonosulfonate, sodium metabenzene disulfonate, the sodium salts of 1,5-naphthalene disulfonic acid and of 2,7-naphthalene disulfonic acid, p-toluenesulfonamide, benzene monosulfonamide, p-chlorobenzene-sulfonamide, xylene sulfonamide, 2,4,6-trichlorodibenzene-sulfonamide, o-benzoyl sulfonimide, o-toluene sulfonimide, diphenylsulfone, thiophene sulfonic acid, allyl sulfonic acid, vinyl sulfonic acid, benzene sulfinic acid and p-toluene sulfinic acid. Such organic sulfur- and oxygen-containing compound brighteners are plating solution-soluble and are utilized in the nickel electroplating baths herein in amounts usually within the range from about 0.1 to 25 grams per liter, preferably from about 0.2 to 7 grams per liter.

The following Examples I-VII in the table hereafter set forth and Examples VIII-XXIII which follow the table are illustrative and non-restrictive of aqueous nickel electroplating baths of this invention which achieve bright level nickel electrodeposits. The numerical values in Examples I-VII in the table designate grams per liter for the nickel salts, grams per liter for the  $H_3BO_3$ , grams per liter for the saccharin, grams per liter for the organic sulfur- and oxygen-containing compound brightener cooperative with the brightener additive compound of this invention, grams per liter for the sodium lauryl sulfate, and milligrams per liter for the brightener additive compounds, i.e. the Type I and/or Type II reaction product, of this invention. The sodium lauryl sulfate is an anti-pitting agent, and the saccharin is a bath stabilizer.

| Nickel Electroplating Bath                                                                                             | Example |       |       |       |       |       |       |
|------------------------------------------------------------------------------------------------------------------------|---------|-------|-------|-------|-------|-------|-------|
|                                                                                                                        | I       | II    | III   | IV    | V     | VI    | VII   |
| $NiSO_4 \cdot 7H_2O$                                                                                                   | 330     | 330   | 330   | 300   | 250   | 300   | 300   |
| $NiCl_2 \cdot 6H_2O$                                                                                                   | 80      | 80    | 40    | 100   | 250   | 80    | 80    |
| $H_3BO_3$                                                                                                              | 40      | 40    | 30    | 40    | 40    | 40    | 40    |
| Saccharin                                                                                                              | 0.5     | 0.5   | 0.1   | 0     | 0.5   | 0     | 0     |
| Organic sulfur- and oxygen-containing compound brightener cooperative with the Type I and/or Type II brightener herein | 0.5     | 0.5   | 0.6   | 0.6   | 0.2   | 0     | 0     |
| Sodium lauryl sulfate                                                                                                  | 0.2     | 0.2   | 0.3   | 0.5   | 0.4   | 0.2   | 0.5   |
| pH                                                                                                                     | 4.0     | 4.5   | 4.0   | 3.8   | 4.0   | 4.0   | 4.0   |
| Temperature, °C                                                                                                        | 60      | 50    | 55    | 65    | 60    | 60    | 60    |
| Type I and/or Type II product of reaction of chloral with $\alpha$ -methylpyridine                                     | 20      | ----- | ----- | ----- | ----- | ----- | 10    |
| Type I and/or Type II product of reaction of propargylic aldehyde with $\alpha$ -methylpyridine                        | 50      | 40    | ----- | ----- | ----- | ----- | 20    |
| Type I and/or Type II product of reaction of furfural with $\alpha$ -methylpyridine                                    | -----   | ----- | 30    | ----- | ----- | ----- | 10    |
| Type I and/or Type II product of reaction of chloral with $\alpha$ -methylpyridine                                     | -----   | ----- | 60    | ----- | ----- | ----- | 10    |
| Type I and/or Type II product of reaction of propargylic aldehyde with $\alpha$ -methylpyridine                        | 20      | ----- | 80    | ----- | ----- | ----- | 20    |
| Type I and/or Type II product of reaction of furfural with $\alpha$ -methylpyridine                                    | -----   | ----- | 100   | ----- | ----- | ----- | 10    |
| Type I and/or Type II product of reaction of chloral with 2-methylquinoline                                            | -----   | ----- | 60    | ----- | ----- | ----- | 10    |
| Type I and/or Type II product of reaction of propargylic aldehyde with 2-methylquinoline                               | -----   | ----- | 30    | 50    | ----- | ----- | 10    |
| Type I and/or Type II product of reaction of furfural with 2-methylquinoline                                           | -----   | ----- | 50    | 20    | ----- | ----- | ----- |

30

35 The organic sulfur- and oxygen-containing compound brightener cooperative with the Type I and/or Type II brightener herein of Examples I-VII of the table and of Examples VIII-XXIII hereafter set forth is the condensation reaction product of the bis(hydroxyethyl)ether of 40 2-butyne-1,4-diol and naphtho-1,8-sultone disclosed in pending U.S. Patent application Ser. No. 500,462, filed Oct. 1, 1965. In place of this cooperating brightener, however, any of the other cooperating brighteners previously disclosed herein can be utilized with good results. The use in Examples I-XXIII of an anti-pit such as sodium 45 benzenemonosulfonate, sodium metabenzene disulfonate, the sodium salts of 1,5-naphthalene disulfonic acid and of 2,7-naphthalene disulfonic acid, p-toluenesulfonamide, benzene monosulfonamide, p-chlorobenzene-sulfonamide, xylene sulfonamide, 2,4,6-trichlorodibenzene-sulfonamide, o-benzoyl sulfonimide, o-toluene sulfonimide, diphenylsulfone, thiophene sulfonic acid, allyl sulfonic acid, vinyl sulfonic acid, benzene sulfinic acid and p-toluene sulfinic acid. Such organic sulfur- and oxygen-containing compound brighteners are plating solution-soluble and are utilized in the nickel electroplating baths herein in amounts usually within the range from about 0.1 to 25 grams per liter, preferably from about 0.2 to 7 grams per liter.

45 The use in such examples of saccharin is also preferred but not essential.

#### EXAMPLE VIII

|                                                                                                                        |                  |     |
|------------------------------------------------------------------------------------------------------------------------|------------------|-----|
| $NiSO_4 \cdot 7H_2O$                                                                                                   | grams/liter      | 330 |
| $NiCl_2 \cdot 6H_2O$                                                                                                   | do               | 80  |
| $H_3BO_3$                                                                                                              | do               | 40  |
| Saccharin                                                                                                              | do               | 0.5 |
| Organic sulfur- and oxygen-containing compound brightener cooperative with the Type I and/or Type II brightener herein | grams/liter      | 0.5 |
| Sodium lauryl sulfate                                                                                                  | do               | 0.2 |
| Type I and/or Type II product of reaction of acetaldehyde with $\alpha$ -methylpyridine                                | milligrams/liter | 50  |

#### EXAMPLE IX

|                                                                                                                        |                  |     |
|------------------------------------------------------------------------------------------------------------------------|------------------|-----|
| $NiSO_4 \cdot 7H_2O$                                                                                                   | grams/liter      | 330 |
| $NiCl_2 \cdot 6H_2O$                                                                                                   | do               | 80  |
| $H_3BO_3$                                                                                                              | do               | 40  |
| Saccharin                                                                                                              | do               | 0.5 |
| Organic sulfur- and oxygen-containing compound brightener cooperative with the Type I and/or Type II brightener herein | grams/liter      | 0.5 |
| Sodium lauryl sulfate                                                                                                  | do               | 0.2 |
| Type I and/or Type II product of reaction of butyraldehyde with $\alpha$ -methylpyridine                               | milligrams/liter | 35  |

75

**13**  
EXAMPLE X

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 300 |
| NiCl <sub>2</sub> ·6H <sub>2</sub> O                                                                                         | do               | 100 |
| H <sub>3</sub> BO <sub>3</sub>                                                                                               | do               | 40  |
| Organic sulfur- and oxygen-containing compound<br>brightener cooperative with the Type I and/or<br>Type II brightener herein | grams/liter      | 0.6 |
| Sodium lauryl sulfate                                                                                                        | do               | 0.5 |
| Type I and/or Type II product of reaction of valeral-<br>dehyde with $\alpha$ -methylpyridine                                | milligrams/liter | 45  |

## EXAMPLE XI

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or<br>Type II brightener herein | grams/liter      | 0.5 |
| Sodium lauryl sulfate                                                                                                        | do               | 0.2 |
| Type I and/or Type II product of reaction of ac-<br>rolein with $\alpha$ -methylpyridine                                     | milligrams/liter | 60  |

## EXAMPLE XII

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or<br>Type II brightener herein | grams/liter      | 0.5 |
| Sodium lauryl sulfate                                                                                                        | do               | 0.2 |
| Type I and/or Type II product of reaction of croton-<br>aldehyde with $\alpha$ -methylpyridine                               | milligrams/liter | 40  |

## EXAMPLE XIII

|                                                                                             |                  |     |
|---------------------------------------------------------------------------------------------|------------------|-----|
| NiSO <sub>4</sub> ·7H <sub>2</sub> O                                                        | grams/liter      | 300 |
| NiCl <sub>2</sub> ·6H <sub>2</sub> O                                                        | do               | 80  |
| H <sub>3</sub> BO <sub>3</sub>                                                              | do               | 40  |
| Sodium lauryl sulfate                                                                       | do               | 0.5 |
| Type I and/or Type II product of reaction of tigal-<br>dehyde with $\alpha$ -methylpyridine | milligrams/liter | 100 |

## EXAMPLE XIV

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of gly-<br>colaldehyde with $\alpha$ -methylpyridine                               | milligrams/liter | 150 |

## EXAMPLE XV

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of suc-<br>inaldehyde with $\alpha$ -methylpyridine                                | milligrams/liter | 175 |
|                                                                                                                              |                  | 75  |

**14**  
EXAMPLE XVI

|                                                                                            |                  |     |
|--------------------------------------------------------------------------------------------|------------------|-----|
| NiSO <sub>4</sub> ·7H <sub>2</sub> O                                                       | grams/liter      | 300 |
| NiCl <sub>2</sub> ·6H <sub>2</sub> O                                                       | do               | 80  |
| H <sub>3</sub> BO <sub>3</sub>                                                             | do               | 40  |
| Sodium lauryl sulfate                                                                      | do               | 0.2 |
| Type I and/or Type II product of reaction of citro-<br>nella with $\alpha$ -methylpyridine | milligrams/liter | 190 |

## EXAMPLE XVII

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 300 |
| NiCl <sub>2</sub> ·6H <sub>2</sub> O                                                                                         | do               | 100 |
| H <sub>3</sub> BO <sub>3</sub>                                                                                               | do               | 40  |
| Organic sulfur- and oxygen-containing compound<br>brightener cooperative with the Type I and/or Type<br>II brightener herein | grams/liter      | 0.6 |
| Sodium lauryl sulfate                                                                                                        | do               | 0.5 |
| Type I and/or Type II product of reaction of pro-<br>pionaldehyde with 2-methylquinoline                                     | milligrams/liter | 35  |

## EXAMPLE XVIII

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of buty-<br>raldehyde with 2-methylquinoline                                       | milligrams/liter | 75  |

## EXAMPLE XIX

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of acro-<br>lein with 2-methylquinoline                                            | milligrams/liter | 60  |

## EXAMPLE XX

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of croton-<br>aldehyde with 2-methylquinoline                                      | milligrams/liter | 80  |

## EXAMPLE XXI

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of tigal-<br>aldehyde with 2-methylquinoline                                       | milligrams/liter | 120 |

15

## EXAMPLE XXII

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of glycol-<br>aldehyde with 2-methylquinoline                                      | milligrams/liter | 130 |

## EXAMPLE XXIII

|                                                                                                                              |                  |     |
|------------------------------------------------------------------------------------------------------------------------------|------------------|-----|
| NiSO <sub>4</sub> ·7H <sub>2</sub> O                                                                                         | grams/liter      | 330 |
| NiCl <sub>2</sub> ·6H <sub>2</sub> O                                                                                         | do               | 80  |
| H <sub>3</sub> BO <sub>3</sub>                                                                                               | do               | 40  |
| Saccharin                                                                                                                    | do               | 0.5 |
| Organic sulfur- and oxygen-containing compound<br>brightener cooperative with the Type I and/or Type<br>II brightener herein | grams/liter      | 0.5 |
| Sodium lauryl sulfate                                                                                                        | do               | 0.2 |
| Type I and/or Type II product of reaction of succin-<br>aldehyde with 2-methylquinoline                                      | milligrams/liter | 90  |

The aqueous baths of Examples I-XXIII supra are utilizable for electrodepositing bright level nickel deposits which are firmly adherent deposits under the plating conditions including current density, bath temperature and pH previously set forth herein.

What is claimed is:

1. A nickel electroplating bath comprising an acidic aqueous solution of at least one nickel salt from the group consisting of the sulfate and chloride of nickel and an effective amount as brightener and leveler of at least one nuclear substituted nitrogen-containing heterocyclic compound selected from the group consisting of those of the formulae:



and



wherein R is selected from the group consisting of lower alkyl, alkenyl, lower alkynyl, hydroxymethyl, trichloromethyl, furfuryl and carboethyl.

R<sub>1</sub> and R<sub>2</sub> separately are each hydrogen and taken together are:



and m is an integer from 0 to 1, m being zero when R<sub>1</sub> and R<sub>2</sub> taken together are as aforesaid, all substituents of said nuclear-substituted heterocyclic compound being linked to carbon atoms of the heterocyclic nucleus.

2. The solution of claim 1 wherein the R-containing substituent of the nuclear-substituted nitrogen-containing compound is linked to the alpha or gamma ring carbon atom relative to the ring nitrogen atom, and the methyl group substituent when present is linked to the alpha or gamma ring carbon atom not linked to said R-containing substituent.

16

3. The solution of claim 2 further characterized by containing another brightening agent which cooperates with the first-mentioned brightening agent, said other brightening agent being an organic sulfur- and oxygen-containing compound brightener selected from the group consisting of aryl sulfonic acids, aryl sulfonates, aryl sulfonamides, aryl sulfonimides, mononuclear aryl sulfonic acids, unsaturated aliphatic sulfonic acids, thiophene sulfonic acid and diphenyl sulfone.

4. The solution of claim 3 wherein R of the formulae is lower alkynyl.

5. The solution of claim 4 wherein R of the formulae is propargyl.

6. The solution of claim 3 further characterized by containing both nickel sulfate and nickel chloride in the solution.

7. The solution of claim 6 further characterized by containing a buffering agent therein.

8. The solution of claim 7 wherein the buffering agent is boric acid.

9. The solution of claim 3 wherein the substituted nitrogen-containing heterocyclic compound is present in the solution in amount of about 5-200 milligrams per liter.

10. The solution of claim 3 wherein R of the formulae is lower alkyl.

11. The solution of claim 3 wherein R of the formulae is alkenyl.

12. A method for electroplating bright nickel deposits comprising passing a current through an acidic nickel plating bath between an anode and cathode, the nickel bath comprising an acidic aqueous solution of at least one nickel salt selected from the group consisting of the sulfate and chloride of nickel, and an effective amount as brightener and leveler of at least one nuclear-substituted nitrogen-containing heterocyclic compound selected from the group consisting of those of the formulae:



and



wherein R is selected from the group consisting of lower alkyl, alkenyl, lower alkynyl, hydroxymethyl, trichloromethyl, furfuryl and carboethyl, R<sub>1</sub> and R<sub>2</sub> separately are each hydrogen and taken together are:



and m is an integer from 0 to 1, m being zero when R<sub>1</sub> and R<sub>2</sub> taken together are as aforesaid, all substituents of said nuclear-substituted heterocyclic compound being linked to carbon atoms of the heterocyclic nucleus.

13. The method of claim 12 wherein the R-containing substituent of the nuclear-substituted nitrogen-containing compound is linked to the alpha or gamma ring carbon atom relative to the ring nitrogen atom, and the methyl group substituent when present is linked to the alpha or gamma ring carbon atom not linked to said R-containing substituent.

14. The method of claim 13 wherein the nickel plating bath contains another brightening agent which cooper-

17

ates with the first-mentioned brightening agent, said other brightening agent being an organic sulfur- and oxygen-containing compound brightener selected from the group consisting of aryl sulfonic acids, aryl sulfonates, aryl sulfonamides, aryl sulfonimides, mononuclear aryl sulfonic acids, unsaturated aliphatic sulfonic acids, thiophene sulfonic acid and diphenyl sulfone.

15. The method of claim 14 further characterized by the nickel plating bath containing both nickel sulfate and nickel chloride.

16. The method of claim 14 wherein R of the formulae is lower alkynyl and the nuclear substituted heterocyclic nitrogen-containing compound is selected from the group consisting of  $\alpha$ -methylpyridine,  $\gamma$ -methylpyridine and 2-methylquinoline.

17. The method of claim 16 wherein R of the formulae is propargyl.

18. The method of claim 14 wherein R of the formulae is lower alkyl.

19. The method of claim 14 wherein R of the formulae is alkenyl.

20. The solution of claim 3 wherein the said first-mentioned brightening agent is at least one compound selected from the group consisting of those of the formulae:



and



21. The solution of claim 3 wherein the said first-mentioned brightening agent is at least one compound selected from the group consisting of those of the formulae:



and



22. The solution of claim 3 wherein the said first-mentioned brightening agent is at least one compound selected from the group consisting of those of the formulae:



and



3,484,345

18

23. The solution of claim 3 wherein the said first-mentioned brightening agent is at least one compound selected from the group consisting of those of the formulae:

5



and



15

24. The solution of claim 3 wherein the said first-mentioned brightening agent is at least one compound selected from the group consisting of those of the formulae:

20



25

and



30

25. The solution of claim 3 wherein said first-mentioned brightening agent is at least one compound selected from the group consisting of those of the formulae:

40



45 and

50



26. The solution of claim 9 wherein the organic sulfur- and oxygen-containing compound brightener is present therein in amount from about 0.1 to 25 grams per liter.

27. The solution of claim 26 wherein the organic sulfur- and oxygen-containing compound brightener is present therein in amount from about 0.2 to 7 grams per liter.

#### References Cited

#### UNITED STATES PATENTS

|           |         |                    |            |
|-----------|---------|--------------------|------------|
| 2,427,286 | 9/1947  | Knapp et al. ----- | 260—283 XR |
| 2,647,866 | 8/1953  | Brown -----        | 204—49     |
| 2,863,802 | 12/1958 | Pyne -----         | 260—297 XR |
| 2,962,498 | 11/1960 | White et al.       |            |
| 3,262,906 | 7/1966  | Perry -----        | 260—283 XR |
| 3,371,096 | 2/1968  | Brust et al. ----- | 260—297 XR |
| 3,400,126 | 9/1968  | Brust et al. ----- | 260—297 XR |

#### FOREIGN PATENTS

|         |        |                |
|---------|--------|----------------|
| 897,401 | 5/1962 | Great Britain. |
|---------|--------|----------------|

UNITED STATES PATENT OFFICE  
CERTIFICATE OF CORRECTION

Patent No. 3,484,345

December 16, 1969

Raymond F. Nambride

It is certified that error appears in the above identified patent and that said Letters Patent are hereby corrected as shown below:

Column 1, lines 36 to 40, that portion of the formula reading " $=\text{CH}_3$ " should read  $-\text{CH}_3$ ; lines 68 to 71,



should read



Column 6, line 61, " $\alpha$ -methylpyridine" should read  $\gamma$ -methylpyridine. Column 7, line 14, " $\alpha$ -methylpyridine" should read  $\gamma$ -methylpyridine; lines 22 to 27, cancel the formula; lines 28 to 32, that portion of the formula reading " $-\text{CH}_2\text{CHOCHCH}_2(\text{CH}_3)-\text{CHCH}_2\text{CH}_2\text{CH}_2(\text{CH}_3)\text{C}=\text{CH}_2$ " should read  $-\text{CH}_2\text{CHOCHCH}_2(\text{CH}_3)\text{CHCH}_2\text{CH}_2\text{CH}_2(\text{CH}_3)\text{C}=\text{CH}_2$ ; lines 44 to 48, that portion of the formula reading " $-\text{CH}=\text{CHCH}_2(\text{CH}_3)\text{CHCH}_2\text{CH}_2\text{CH}=(\text{CH}_3)_2$ " should read  $-\text{CH}=\text{CHCH}_2(\text{CH}_3)\text{CHCH}_2\text{CH}_2\text{CH}=\text{C}(\text{CH}_3)_2$ ; line 61, " $\alpha$ -methylpyridine" should read  $\gamma$ -methylpyridine. Column 15, line 54, "carboethyl" should read carboethyl. Column 16, lines 45 to 49, the formula should appear as shown below:



3,484,345  
(2)

Column 3, lines 27 to 30, the formula should appear as shown below



Column 17, line 12, "alkynyl and the nuclear substituted heterocyclic nitrogen-containing compound is selected from the group consisting of  $\alpha$ -methylpyridine,  $\gamma$ -methylpyridine and 2-methylquinoline." should read -- alkynyl. --.

Signed and sealed this 3rd day of November 1970.

(SEAL)  
Attest:

EDWARD M. FLETCHER, JR.  
Attesting Officer

WILLIAM E. SCHUYLER, JR.  
Commissioner of Patents